

## UNITED STATES PATENT OFFICE

EUGENE FITZPATRICK, OF WOODHAVEN, CHARLES W. CLARK, OF BELLEROSE, AND PETER A. TIERNAN, OF LAUREL HILL, NEW YORK, ASSIGNEES TO NICHOLS COPPER COMPANY, OF NEW YORK, N. Y., A CORPORATION OF NEW YORK

## METHOD OF PRODUCING METALLIC POWDERS

No Drawing.

Application filed June 20, 1928. Serial No. 287,083.

This invention relates to method of making metallic powders, and more particularly to relatively pure fine metallic powders.

The invention has proven to be of great merit more specifically in the production of copper powder and has produced fine copper powder of a high degree of purity.

Many uses are well known to those skilled in this art for metallic powders, and more particularly for relatively pure fine metallic powders.

By way of example, the use of fine copper powder is well known to those skilled in the art, for example as in paints, lacquers, for plating, for copper carbon brushes, and other uses. In many of these uses it is desirable to have a product of the highest degree of purity compatible with its economical production, and which will contain no extraneous or altered coating as a protecting medium or as oxidation. One of the great difficulties experienced in making such a product has been in producing a copper powder free from oxidation and other impurities.

An object of the present invention is to produce fine metallic powders of an extremely high degree of purity, and in a highly satisfactory commercial manner. More specifically an object of the invention is to produce fine metallic copper of a very high degree of purity.

Further objects of the invention will more fully appear from the following description illustrating by way of example the preferred method of carrying out the same.

The invention consists in the method herein described in accordance with certain preferred embodiments thereof, and the invention will be more particularly pointed out in the appended claims.

Broadly speaking, the method consists in three steps: (1) formation in an electrolytic cell, (2) washing free from the electrolyte, and (3) drying. Since suitable apparatus well known in the art may be adapted for carrying out the method, and since such apparatus per se forms no part of the present invention, it is believed that the method will be clearly understood, by those skilled

in the art, without showing the apparatus, and hence the apparatus will not be illustrated.

The production of fine metallic powders is well known in the art, and it has long been desired to produce such powders in as pure a state as possible. The present method is an improvement over prior processes, and by its use metallic powders, such for example as copper powder, averaging 99.56% purity and as high as 99.75% purity have been produced.

As illustrative of the invention the method of producing copper powder will be described in detail; it being understood that the invention is not thereby to be limited to this specific material.

## Formation in electrolytic cell

A suitable electrolyte, such as copper sulfate, is placed in an electrolyte tank, such for example as a wooden tank lined with sheet lead. An anode of copper, preferably in plate form, is suitably suspended in the electrolyte, and a cathode of copper, preferably in rod or bar form, is similarly suspended in the electrolyte; and the anode and cathode are respectively connected to the plus and minus sides of a suitable source of electric current. The relative size of the electrodes are so proportioned with respect to the current used, that the current density at the cathode will be high; the purpose being to use such a current density that the copper particles deposited on the cathode will be of the desired degree of fineness and will form thereon in a loose fluffy mass, such as in the form of a metal sponge or slime, which will be easily dislodged from the cathode and in which the separate particles remain only loosely adherent. The metal sponge or slime is freed from the cathodes as by rapping or jarring the cathodes at frequent intervals to thereby dislodge the sponge or slime and precipitate the same in the bottom of the tank.

## Washing free from electrolyte

The precipitate is now removed from the electrolyte in a suitable manner, together with a small amount of electrolyte serving

to prevent oxidation, and is freed of the electrolyte, such for example as by means of a gravity filter and circulating water, during which time the copper particles are always 5 kept submerged, or substantially protected by the liquid, to prevent oxidation. During the washing or cleansing of the particles the temperature of the liquid should be so regulated or limited that the washing liquid never 10 exceeds about 120° F. The washing should be done preferably with boiled water, condensate, or suitable liquid of a non-oxidizing character; in order that the particles will not be oxidized thereby or their purity in any 15 way affected.

#### Drying

The washed particles are now placed in suitable receptacles, such for example as shallow copper pans, with the particles substantially submerged. The pans are placed in a cold vacuum dryer of suitable type, the dryer closed and evacuated to a suitable degree, such as to carry away subsequently released 20 volatile matter without injuriously affecting the particles, such as by oxidation, and the dryer then heated to a point sufficient to evaporate the liquid, and preferably to the boiling point of the liquid. This method of 25 protecting the particles against oxidation or 30 impurities is very important, if not essential. The copper particles are left in the dryer until substantially entirely dried. The powder is then removed, and screened to the 35 desired fineness.

In order that those skilled in the art may more fully appreciate the invention, and the beneficial results obtained thereby, we will give following a brief example of a run actually carried on under practical commercial 40 conditions in connection with producing copper powder. While this is not to be taken in a limiting sense, nevertheless it is thought that it may be of assistance in understanding 45 the invention and in serving as an illustration of one preferred embodiment of the invention.

*Example.*—The tank used was constructed of wood lined with sheet lead. The inside 50 dimensions were 36" by 18" by 36" depth at one end and 40" depth at the other end. A 4" outlet was placed at the lower end for removal of the precipitate. The anodes consisted of six copper plates each 12" wide and 55 submerged 24" below the surface of the electrolyte; thereby providing an anode surface of 12 square feet. The cathodes consisted of 12 copper rods each 3/8" in diameter and submerged 24" in the electrolyte; thereby providing 60 a cathode surface of approximately 2.356 square feet. The anodes and the cathodes were connected respectively in multiple; and were connected to a suitable source of electric current. The electrolyte varied in 65 composition from 2.29% to 2.45% of copper

(as copper sulphate) and from 11.32% to 11.43% sulphuric acid.

The cell was operated for 90 hours, and the average current used was 893.75 amperes at 1.50 volts, with the average electrolyte temperature at 129.3° F. The current density at the anodes averaged approximately 74.48 amperes per square foot; while the current density at the cathodes averaged approximately 379.35 amperes per square foot. No artificial circulation was used in the cell; the only circulation being that caused by gassing at the electrodes. The cathodes were rapped every 15 minutes to dislodge the copper sponge or slime and the cell was shut down once each day to clean out the precipitate from the bottom of the tank.

The copper slime or sponge thus removed was placed in a gravity filter and washed free from the electrolyte by circulating water through it; care being taken to keep the finely divided copper particles submerged to prevent oxidation. The washing was continued until the water showed no trace of sulphates, this being determined by testing 85 with barium chloride.

It has been found to be highly desirable, if not essential, that the temperature of the water used for washing should be kept below 120° F., as above this temperature considerable oxidation takes place; and likewise it has been found that boiled water or condensate should be used for washing.

The washed material was placed in copper pans, in a layer of 1/2" thickness and with 1/2" water standing above it. The pans were then placed in a cold vacuum dryer, the dryer closed and the vacuum brought up to about 26" of mercury. After this vacuum had been reached, the steam was turned on and the temperature of the dryer was brought to the boiling point of the water, which at this pressure was about 125° F. This method of keeping the material covered with water before drying is likewise deemed to be very desirable, if not essential. In order to prevent oxidation extreme care was taken to keep the material at all times free from contact with air above 110° F.; and therefore for this and other reasons the dryer was evacuated before the temperature of the material was raised. By noting when the formation of condensate stopped in the vacuum dryer condensers it was determined when the material was completely dried.

The material was then removed from the vacuum dryer and the finely divided copper powder thus produced was screened through a 160 mesh screen. The material which passed the screen amounted to 175 lbs. The resultant product averaged 99.56% purity, and in some instances was as high as 99.75% pure. The resulting product of pure finely divided copper particles is not easily suscep- 125 130

tible to atmospheric oxidation when in dry form and is therefore quite stable; being also free from any extraneous substance.

The theoretical amount of finely divided copper in pounds which can be produced by 5 the ampere hours used is:

$$893.75 \times \frac{1.186}{453.6} \times 90 = 210.3$$

10 The ampere efficiency for this run, based on good production, was,—

$$\frac{175}{210.3} = 83.2\%$$

15 The powder used in this run in kilowatt days was,—

$$\frac{893.75 \times 1.50}{1,000} \times \frac{90}{24} = 5.02.$$

20 This is 2.87 kilowatt days per 100 pounds of copper powder produced.

While certain minor changes may be made in the method without departing from the spirit or scope of the invention, as will be 25 well understood by those skilled in the art; nevertheless, it might be pointed out that, in addition to the features of importance enumerated heretofore, there are certain factors which are believed to be of importance, and 30 such of these factors as we deem of importance at this time will be pointed out following. It would appear that the metal sponge or slime produced should be taken from the metallic anode of the corresponding metal, 35 and that the cathode should be of the same metal; to preclude any opportunity of impurities entering into the product. We have found that it is desirable to keep the copper content of the electrolyte substantially within 1% variation, and the acid content of the 40 electrolyte within 5% variation. We have further found that although the current density heretofore disclosed is satisfactory, nevertheless much higher current densities may be successfully employed. The electrolyte 45 and anode should be free from harmful impurities, such for example as arsenic, antimony, bismuth and lead.

Having thus described our invention with 50 particularity with reference to the preferred method of carrying out the same, it will be obvious to those skilled in the art, after understanding our invention, that various changes and modifications may be made there- 55 in without departing from the spirit and scope of our invention, and we aim in the appended claims to cover such changes and modifications as are within the scope of the invention.

60 What we claim is:

1. Method of producing metal powder, which comprises disintegrating a metal by electrolysis to produce relatively fine metallic particles, removing the metallic particle precipitate from the electrolyte while pre-

venting oxidation, washing said precipitate free from said electrolyte, and introducing said particles, submerged in a non-oxidizing medium, into a suitable vacuum dryer before the latter has been substantially heated, 70 while maintaining said particles free from oxidation, creating a vacuum in said dryer, and thereafter heating said dryer to thereby cause said medium to evaporate and said particles to be dried.

2. Method of producing metal powder, which comprises electrolytically disintegrating a metal to produce relatively fine pure metallic particles, maintaining said particles free from atmospheric contact and while so maintained washing them free from the electrolyte and submerging in a non-oxidizing medium, placing said submerged particles in vacuo and evaporating said medium while maintaining sufficient vacuum to rapidly remove all volatile matter and until said particles are dry, to thereby prevent oxidation of said particles.

3. Method of producing copper powder, which comprises electrolytically disintegrating substantially pure metallic copper to produce relatively fine copper particles, maintaining said particles free from atmospheric contact and while so maintained washing them free from the electrolyte and submerging in water, placing said submerged particles in vacuo and evaporating said water while maintaining sufficient vacuum to rapidly remove all volatile matter and until said particles are dry, to thereby prevent oxidation of said particles.

4. Method of producing metal powder, which consists in forming metal sponge in an electrolyte, washing said sponge free from said electrolyte to provide substantially pure metal particles, covering said particles with a non-oxidizing liquid, placing said particles thus protected in vacuo, and evaporating said liquid to thereby dry said particles substantially free from oxidation and extraneous matter.

5. Method of producing metal powder, which consists in forming metal sponge in an electrolyte, precipitating said sponge, washing said precipitate free from said electrolyte to provide substantially pure metal particles, covering said particles with water, placing said particles thus protected in vacuo, and evaporating said water to thereby dry said particles substantially free from oxidation.

6. Method of producing metal powder, which consists in forming metal sponge in an electrolyte, washing said sponge free from said electrolyte in water to provide substantially pure metal particles, keeping said particles free from oxidation during said washing, and at the end of said washing leaving said particles covered with water, placing said particles thus protected in vacuo, and

evaporating said water to thereby dry said particles substantially free from oxidation.

7. Method of producing metal powder, which consists in forming a metal sponge in an electrolyte, removing said sponge, washing the particles thereof and placing said particles in vacuo while always maintaining said particles submerged in a liquid preventing substantial oxidation, and drying said particles while in vacuo, to thereby produce a substantially non-oxidized fine metal powder free from extraneous matter.

8. Method of producing metal powder, which consists in forming fine metal particles by disintegrating a mass of metal by electrolysis in an electrolyte of the same metal, removing said particles, washing the particles and placing said particles in vacuo while always maintaining said particles submerged in a liquid preventing substantial oxidation, and drying said particles while in vacuo, to thereby eliminate said liquid and produce a substantially non-oxidized pure fine metal powder.

9. Method of producing copper powder, which consists in placing a copper anode and a suitable cathode in a copper sulphate electrolyte, passing a relatively high density electric current of relatively low potential between said electrodes to produce fine particles of copper in said electrolyte, removing and washing said particles free from said electrolyte while keeping said particles submerged to prevent oxidation, and after washing and while still submerged placing said particles in a vacuum dryer, producing a vacuum therein while keeping the temperature below about 120° F., and after said vacuum has been brought up to about 26 inches of mercury increasing the temperature of the dryer to the boiling point of the submerging liquid at the pressure employed and drying said particles in vacuo.

10. Method of producing non-oxidized substantially pure copper powder, which comprises forming copper sponge in an electrolyte, removing said sponge while preventing its exposure to air of a temperature greater than approximately 110° F., washing said sponge free of said electrolyte with water below approximately 120° F., placing said copper submerged in water in suitable receptacles, placing said receptacles in a substantially cool vacuum dryer, creating a vacuum therein of approximately 26 inches of mercury, and thereafter raising the temperature of said dryer up to approximately 125° F., to thereby dry said copper particles and produce copper powder in pure non-oxidized form.

11. Method of producing copper powder of a degree of purity between 99% and 100%, which comprises electrolytically disintegrating copper in a copper sulphate electrolyte to produce fine copper particles, washing said

particles free from said electrolyte with water, covering said particles with water, placing said covered particles in a relatively cool vacuum dryer, evacuating said dryer, and heating said dryer and drying said particles in vacuo, said particles being kept free from contact with air above 110° F. and water above 120° F. at atmospheric pressure from the time of removal from said electrolyte until placed in vacuo.

12. Method of producing fine copper powder of a degree of purity between 99% and 100%, which comprises electrolytically disintegrating copper in a copper sulphate electrolyte with a relatively low anode current density and a relatively high cathode current density, washing said disintegration particles free from said electrolyte with water, covering said particles with water, placing said covered particles in a relatively cool vacuum dryer, evacuating said dryer to approximately 26 inches of mercury, and heating said dryer to approximately 125° F. and drying said particles in vacuo, said particles being kept free from contact with air above 110° F. and water above 120° F. at atmospheric pressure from the time of removal from said electrolyte until placed in vacuo.

In testimony whereof we have signed our names to this specification.

EUGENE FITZPATRICK.  
CHARLES W. CLARK.  
PETER A. TIERNAN.

95

100

105

110

115

120

125

130